

- [54] CATALYTIC REFORMING PROCESS WITH LIQUID PHASE SULFUR REMOVAL

- [75] Inventor: Thomas J. Nelson, Mt. Prospect, Ill.

- [73] Assignee: **Atlantic Richfield Company,**  
**Philadelphia, Pa.**

[ \* ] Notice: The portion of the term of this patent, subsequent to Sep. 30, 1997, has been disclaimed.

[21] Appl. No.: 130,314

[22] Filed: Mar. 14, 1980

#### Related U.S. Application Data

- [63] Continuation-in-part of Ser. No. 9,001, Feb. 5, 1979,  
Pat. No. 4,225,417.

- [51] Int. Cl.<sup>3</sup> ..... C10G 25/00; C10G 23/02  
[52] U.S. Cl. ..... 208/89; 208/91;

- 208/138; 208/139

- [58] **Field of Search** ..... 208/89, 91, 88, 249,  
208/139

[56] References Cited

## U.S. PATENT DOCUMENTS

4,225,417 9/1980 Nelson ..... 208/89

*Primary Examiner*—Curtis R. Davis  
*Attorney, Agent, or Firm*—Stanley M. Wels

[57] ABSTRACT

A reforming process is disclosed which comprises contacting a sulfur-containing hydrocarbon material in at least one liquid phase scavenging or sulfur removal zone with at least one manganese-containing composition at conditions to remove at least a portion of said sulfur from said hydrocarbon material to produce a hydrocarbon feedstock having a reduced concentration of sulfur; and contacting said hydrocarbon feedstock with a catalyst comprising a minor catalytically effective amount of at least one platinum-group metal component, optionally, a major amount of a porous solid support, optionally, a minor catalytically effective amount of at least one halogen component, and optionally, at least one rhenium component in the presence of hydrogen at hydrocarbon reforming conditions to obtain a hydrocarbon reformate product.

## 12 Claims, 5 Drawing Figures



**FIG. I**



FIG. 2





FIG. 3

FIG. 4



FIG. 5

SULFUR REMOVAL VERSUS TRAP TEMPERATURE

## CATALYTIC REFORMING PROCESS WITH LIQUID PHASE SULFUR REMOVAL

### CROSS REFERENCE TO A RELATED APPLICATION

This application is a continuation-in-part of an earlier filed and a co-pending application, Ser. No. 9,001 filed Feb. 5, 1979, now U.S. Pat. No. 4,225,417, the teachings of which are expressly incorporated by reference herein.

### BACKGROUND OF THE INVENTION

#### Field of the Invention

This invention relates to removal of sulfur from a hydrocarbon material. More particularly, this invention relates to the use of a manganese-containing material in the removal of sulfur from hydrocarbon materials and subjecting the resulting reduced sulfur-containing hydrocarbon feedstock to hydrocarbon reforming.

Catalytic hydrocarbon reforming, a method to improve the octane value of a naphtha feedstock, is well known. Many of the catalysts used to carry out such a reforming process tend to be especially sulfur sensitive. Examples of such especially sulfur sensitive reforming catalysts are those employing a platinum-group metal, e.g., platinum, and optionally as a co-metal component, rhenium. Several examples of reforming processes are fixed-bed hydroforming (Standard Oil Development Company, M. W. Kellogg Company, and Standard Oil Company (Indiana)), Platforming (Universal Oil Products Company), Catforming (Atlantic Refining Company), Houdriforming (Houdry Process Corporation), Ultraforming (Standard Oil Company (Indiana)), Rex-forming (Universal Oil Products Company), Power-forming (Esso Research and Engineering Company), Magnaforming (Engelhard Minerals and Chemicals Corporation), and Rheniforming (Chevron Research Company).

Under the high hydrogen partial pressure condition used in catalytic reforming, sulfur compounds are readily converted into hydrogen sulfide which, unless removed, will build up to a high concentration in hydrogen recycle gas. It becomes especially important in view of the high sulfur sensitivity of platinum-group metal reforming catalysts to use feedstocks having reduced sulfur levels, e.g. of less than about 1 ppm. "Reforming" is meant herein and in the claims to be a catalytic process wherein a hydrocarbon feedstock is contacted with a hydrocarbon reforming catalyst in the presence of hydrogen at hydrocarbon reforming conditions to produce at least one reformate product having an increased octane value, e.g., Research Octane Number (RON) relative to that of the hydrocarbon feedstock.

K. E. Louder et al. U.S. Pat. No. 3,898,153 (1975) disclose an improvement in catalytic reforming of naphthas wherein a hydrotreated feedstock is passed through a zinc oxide bed preceded by a chloride scavenging zone. The chloride scavenging zone is necessary because hydrochloric acid gas in the reformer recycle gas reacts with zinc oxide to form zinc chloride. The zinc chloride in turn is carried into the reforming zone where it adversely affects the reforming catalyst.

P. R. Westmoreland et al. in *Environmental Science and Technology*, Volume 11, Pages 488-491, report initial rates for reaction between H<sub>2</sub>S in a mixture of H<sub>2</sub>S and H<sub>2</sub> and MnO<sub>x</sub>, CaO, ZnO and V<sub>2</sub>O<sub>5</sub> over a tempera-

ture range of 570°-1470° F. (300°-800° C.). Manganese oxide was reported to have the highest reaction rate and possessed favorable properties for a high temperature desulfurization process.

5 Removal of sulfur, either from waste gas or industrial exhaust or flue gases, by means of an oxide of manganese is disclosed in the following patents: U.S. Pat. Nos. 3,761,570 (1973), 3,723,598 (1973), 3,492,083 (1970) and British Pat. No. 1,144,071.

10 Removal of sulfur from carbonaceous solid fuels by conversion of sulfur impurities to hydrogen sulfide followed by absorption of the hydrogen sulfide on supported manganese oxide is disclosed in the following U.S. Pat. Nos. 2,927,063 (1960), 2,950,229 (1960), 2,950,231 (1960), and 3,101,303 (1963).

15 Methods for regenerating manganese oxide are disclosed in the following U.S. Pat. Nos. 2,927,063 (1960), 2,950,229 (1960), 3,492,083 (1970) and 3,101,303 (1963).

20 U.S. Pat. No. 4,045,331 (1977) discloses a process for both demetalization and desulfurization of a petroleum feedstock by means of a manganese oxide supported on an alumina.

25 U.S. Pat. No. 3,063,936 (1962) discloses removal of H<sub>2</sub>S produced during a catalytic hydrodesulfurization of a naphtha fraction by contacting the hydrotreated feedstock in the vapor phase at about 662° F. (350° C.) with an absorbing material comprising zinc oxide (reported to be preferred), manganese oxide or iron oxide. The desulfurized naphtha is then used in a steam-reforming process for the production of methanol synthesis gases.

30 U.S. Pat. Nos. 1,840,158 (1932), 2,177,343 (1939), 2,618,586 (1952), 2,314,576 (1943), 2,950,229 (1960), 3,320,157 (1967), and 3,996,130 (1976) all disclose the use of a manganese-containing material to remove at least a portion of a sulfur component contained in a hydrocarbon material. However, none of these references disclose the removal of a sulfur component from a hydrocarbon material in the context of a reforming process. None of the references teach that sufficient removal of sulfur from the hydrocarbon material can be achieved so as to make them useful as feedstocks for a reforming zone. In summary, a teaching that the sulfur content of a hydrocarbon material can be reduced by means of a process employing a manganese-containing composition does not disclose nor teach that such removal is necessarily sufficient to permit use of such a process upstream from a reforming zone.

35 U.S. Pat. No. 4,155,835 (1979) discloses a process for desulfurizing a naphtha or other hydrocarbon fractions boiling below about 430° F. which is accomplished by cascading such a sulfur-containing material with added hydrogen over a combination of desulfurizing catalyst, under appropriate process conditions, and thereafter

40 passing the total effluent, over a massive catalyst comprising zinc oxide or other suitable metal oxides. A desulfurized effluent from the above process can then be again reformed with a by-mettallic catalyst. Other 45 suitable metal oxides, other than zinc oxide, are broadly suggested, however, no specific examples of such other metal oxides are disclosed nor any criteria for selecting them.

45 Many of the cited references suggest that zinc oxide and manganese oxide are equally effective and can be used interchangeably. This teaching is misleading when halides are present. For example, none of the references teach or suggest that where halogen-containing com-

pounds are present and can both contact and react with the material for removing sulfur, a means for scavenging halide, required in the case of zinc oxide, is not required in the case of manganese oxide. Halogen-containing compounds are often present in the hydrocarbon feedstock, the hydrogen recycle line, and/or the reforming zone due to addition of halogen-containing compounds into any and all of these in order to maintain the halogen content on a, e.g., platinum-group metal containing, reforming catalyst.

U.S. Pat. No. 2,922,756 (1960) discloses an endothermic reforming process for a sulfur-containing feedstock. Of critical importance to the invention disclosed in U.S. Pat. No. 2,922,756 is that a portion of the heat to carry out the endothermic process is derived from a heat transfer effected directly within the catalyst bed in a reaction zone. The selected material must have sufficient desulfurization qualities to remove sulfur in a moving bed configuration. Further, the material must be able to form a sulfide at specified conditions, but which will oxidize at other selected conditions in a heating zone and further be reduced by hydrogen or hydrocarbons. These materials must, of course, be heat retentive. Materials asserted to fulfill the above requirements include iron, nickel, cobalt, molybdenum, vanadium, manganese and mixtures thereof. That manganese can be used interchangeably and with equal effectiveness with the other cited materials in a moving or fluidized bed for the purpose of removing sulfur from a hydrocarbon material which is later to be reformed is a misleading teaching when applied to a fixed bed sulfur removal zone. It has been discovered that in a fixed bed configuration oxides of manganese perform in a surprisingly very superior fashion to the other oxides. The superior performance of oxides of manganese is discussed in more detail hereinafter.

As a reactant, manganese oxide has a significantly greater propensity than zinc oxide to absorb or react with hydrochloric acid under the following process conditions: temperature in the range 600° to 1000° F. (316° to 538° C.) preferably 650° to 850° F. (343° to 454° C.), pressure in the range 150-750 psig., a hydrogen concentration in the range 1/1 to 30/1 moles of hydrogen per mole of hydrocarbon, and a space velocity (vhs) in the range 500-50,000 vol. of gas/hour/vol. of reactant.

It has been found that a manganese component, preferably a manganese oxide, will scavenge hydrogen sulfide significantly more effectively than zinc oxide as shown in Example 3. Further, it has been discovered surprisingly that unlike zinc oxide, manganese in the form of an oxide, halide or sulfide has a negligible, if any, adverse affect on a platinum-group metal reforming catalyst after an activation-regeneration cycle as shown in Example 5.

It has been discovered surprisingly that manganese oxide in the liquid phase has a superior ability to remove mercaptans from a hydrocarbon material than does zinc oxide in the liquid phase.

One difficulty with manganese-containing material for use in a sulfur removal zone is their tendency to give up hydrogen sulfide in the presence of water vapor. Clearly, the evolution of even small amounts of hydrogen sulfide, e.g., 3 ppm, can severely poison sensitive platinum-rhenium reforming catalysts. A source of such water vapor is often the recycled gas which leaves a reforming zone. We have found that liquid phase opera-

tion can permit easy isolation from such recycled gas as is shown in FIG. 2 at location E.

#### BRIEF DESCRIPTION OF THE INVENTION

- It is an object of this invention to provide a method for the effective removal of sulfur from sulfur-containing hydrogen and/or hydrocarbon materials, to produce hydrogen and/or hydrocarbon feedstocks having reduced sulfur content for a reforming process which utilizes a sulfur sensitive catalyst. It is an object of this invention to provide a hydrocarbon reforming process involving sulfur removal from hydrogen and/or hydrocarbon materials which achieves improved results relative to prior art processes involving sulfur removal with zinc oxide.
- It is an object of this invention to provide a method for the effective removal of sulfur from sulfur-containing hydrocarbon materials by means of a liquid phase removal zone employing a manganese-containing component to produce feedstocks for a reforming process which utilizes a highly sulfur sensitive catalyst. It is an object of this invention to provide the following benefits which accrue from a liquid phase sulfur removal zone: (1) it, the zone, both can be isolated from the gas recycled from reforming zone and is more easily isolated from regeneration and/or reactivation processes; (2) it avoids the presence of partial pressures of water which can cause release of hydrogen sulfide from a sulfided manganese-containing component; (3) it is a substantially smaller removal zone with a correspondingly smaller vessel which can achieve the same results in the liquid phase as can be obtained in the vapor phase; and (4) it provides a process that involves an energy saving, as is clear from the relationship for work, i.e., pressure drop time volume of material.

Other objects of this invention are clear from the specification.

Regeneration throughout this specification and in the claims means the process wherein a portion of carbonaceous deposits on a reforming catalyst are removed by an oxidative burn-off. Carbonaceous deposits can form on a reforming catalyst during reforming of a hydrocarbon feed. Regeneration of a catalyst to remove carbon is relatively quick and used in most commercial catalytic conversion operations.

An example of a conventional coke-burning procedure is one which consists of first purging hydrogen from the catalytic environment either by displacement with an inert gas or by depressurizing the environment containing the catalyst down to a fraction of an atmosphere, or by any other similar procedure. The carbonaceous deposits are then removed by contacting the catalyst with controlled amounts of oxygen typically obtained by mixing together air and an inert gas in such a manner that the temperature of the catalyst does not exceed about 1100° F. This last requirement is necessary in order to avoid detrimental migration or transformations of the platinum-group metal. A concentration of oxygen in the treatment gas is usually adjusted to achieve a combustion temperature in the range of about 700° F. to about 1100° F. and to achieve substantially complete carbon removal. This procedure can be performed at any desired pressure. The time of contact is generally from about 1 to about 12 hours or more depending on the extent of the carbonization of the catalyst.

Reactivation throughout the specification and in the claims means the process wherein a previously regener-

ated catalyst is further treated to disperse or redistribute the supported platinum-group metal and/or to redistribute and recomposite the halogen content of the catalyst to maintain catalytic activity. Examples of U.S. patents disclosing a reactivation procedure are U.S. Pat. Nos. ;B 3,637,524 (1972) and 3,781,219 (1973) both expressly incorporated herein by reference.

The hydrocarbon materials used in the present process comprise hydrocarbon fractions containing naphthenes and paraffins that, preferably boil primarily within the gasoline range. Typically, the hydrocarbon materials used comprise about 20% to about 70% by weight of naphthenes and about 25% to about 75% by weight of paraffins. The preferred hydrocarbons material for use as a feed or chargestock consists essentially of naphthenes and paraffins, although in some cases aromatics and/or olefins may also be present. When aromatics are included, these compounds comprise about 5% to about 25% by weight of the total hydrocarbon material. A preferred class of hydrocarbon feed or chargestock includes straight run gasolines, natural gasolines, synthetic gasolines and the like. On the other hand, it is frequently advantageous to use as hydrocarbon feed or chargestock of thermally or catalytically cracked gasolines or higher boiling fractions thereof, called heavy naphthas. Mixtures of straight run and cracked gasolines can also be used. The gasoline used as hydrocarbon feed or chargestock may be a full boiling range gasoline having an initial boiling point within the range of about 50° F. to about 150° F. (10° C. to 66° C.) and an end boiling point within the range of about 325° F. to about 425° F. (163° C. to 218° C.) or may be a selected fraction thereof which generally will be a higher boiling fraction commonly referred to as a heavy naphtha—for example, a naphtha boiling in the range of a C<sub>7</sub> to about 400° F. (204° C.). In some cases, it is also advantageous to use pure hydrocarbons or mixtures of hydrocarbons that have been extracted from hydrocarbon distillates—for example, straight-chain paraffins—which are to be converted to aromatics.

#### DETAILED DESCRIPTION OF THE INVENTION

Broadly this invention comprises a process for removal of a sulfur component from sulfur-containing hydrogen and/or hydrocarbon material by contacting a manganese-containing material or composition with the hydrogen and/or hydrocarbon material. The manganese component of such a manganese-containing material is present in an effective amount sufficient to provide desired removal of sulfur-containing compounds, such as for example, H<sub>2</sub>S present in the hydrogen and/or hydrocarbon material. The period of contacting is sufficient to permit the desired removal of sulfur-containing compounds from the hydrogen and/or hydrocarbon material. Preferably, the manganese component is combined with a suitable binder or support to make pellets which preferably have sufficient crush strength for the application intended. Examples of suitable binders or supports are clays, graphite, alumina, zirconia, chromia, magnesia, curia, boria, silica-alumina, silica-magnesia, chromia-alumina, alumina-boria, alumina-silica-boron phosphate, silica-zirconia, and alumina and silica combinations.

In one embodiment of this invention, an initial concentration of a sulfur component, calculated as elemental sulfur, in the hydrogen and/or hydrocarbon material to be contacted with the manganese component during

normal operation as opposed to an upset condition is preferably in the range of about 0.1 to about 100 parts per million (ppm) by weight, and more preferably about 0.2 to about 50 ppm by weight. An upset condition occurs when the amount of sulfur-containing components of the hydrogen and/or hydrocarbon material increase to well over 100 ppm by weight, e.g., in excess of 500 ppm by weight. This condition can occur for example, due to malfunction of the sulfur stripping zone of a hydrodesulfurization system. The sulfur component concentration of the hydrogen and/or hydrocarbon material subsequent to being contacted with the manganese-containing material of the present invention is preferably less than about 0.2 ppm by weight and still more preferably less than about 0.1 ppm by weight.

In another embodiment of this invention, a process for reforming a hydrocarbon material containing a sulfur component, such as discussed in the preceding paragraph, comprises: contacting in a liquid phase sulfur removal zone at sulfur removal conditions, said hydrocarbon material with a manganese-containing composition which comprises a manganese component capable of removing at least a portion of said sulfur component at sulfur removal conditions to produce a reduced sulfur-containing hydrocarbon feedstock, and contacting in a reforming zone in the presence of hydrogen at hydrocarbon reforming conditions, said feedstock with a catalyst comprising a catalytically effective amount of a platinum-group metal component capable of reforming said feedstock at such reforming conditions to produce a reformed product.

The term "liquid phase" is intended to mean that during processing the temperature and pressure conditions are adjusted so that there is a hydrocarbon liquid phase present in the sulfur removal zone. Generally, the more hydrocarbon liquid phase present in the sulfur removal zone, the more efficient is the operation for removing sulfur components. However, the precise amount of hydrocarbon liquid phase present is not critical to the operation of the sulfur removal zone. Clearly, the pressure required to maintain a liquid phase will depend upon the temperature for temperatures below the critical temperature of a particular feedstock. It has been found generally that the higher the temperature in the sulfur removal zone, the more effectively are sulfur components, such as mercaptans, removed. This relationship between temperature and sulfur removal is shown in FIG. 5. However, also shown in FIG. 5 is the fact that temperatures much above 700° F. do not result in additional sulfur components being removed, i.e., the maximum of sulfur removal occurs at or before 700° F.

Pressure can be at any value necessary to maintain the presence of a hydrocarbon liquid phase, but is preferably in the range 15 psig to about 800 psig because this is generally the pressure range for the hydrocarbon material, i.e., stripper bottoms, leaving a hydrodesulfurization zone, such as zone 52 of FIG. 1 or zone 2 of FIG. 2, and the pressure in a reforming zone.

Preferably, the temperature of the hydrocarbon feedstock is below the critical temperature of the hydrocarbon feedstock. More preferably, the temperature is in the range of about 400° to about 800° F. and most preferably the temperature is in the range of about 450° to about 700° F.

There are several methods by which a manganese component can be composited with a binder or support. One such method, for example, contemplates impregnating a support in the form of either a pellet or extrud-

ate with an aqueous solution of a manganese salt, such as manganous chloride, manganous nitrate, etc. Comulling methods are equally appropriate; for example, manganese oxide binders can be mulled with a solid binder, such as cited earlier, preferably alumina, with sufficient water and cosolvent, e.g., acetic or nitric acid solutions, to create a paste extrudable through a die.

Alternatively, the binder can be co-mulled with an aqueous solution of a manganese salt until an extrudable paste is formed. By these and other conventional methods, manganese may be composited with the binder or support.

Calcination at a temperature between about 450° and 1600° F. (232° and 870° C.) preferably between 550° and 1000° F. (288° and 538° C.), and more preferably between about 600° and 900° F. (316° and 482° C.) is carried out subsequent to impregnation or comulling of a manganese salt into or with a binder or support, e.g. of alumina. This calcination procedure produces a reactant or manganese-containing material containing one or more of the common oxides of manganese. Examples of such common oxides are MnO, MnO<sub>2</sub>, MnO<sub>3</sub>, Mn<sub>2</sub>O<sub>3</sub>, Mn<sub>2</sub>O<sub>7</sub>, Mn<sub>3</sub>O<sub>4</sub>, and Mn<sub>2</sub>O<sub>4</sub>.

Manganese-containing material when at least a portion thereof is in the form of particles has at least a portion, preferably a majority by weight, of such particles each with an overall average diameter in the range of about  $\frac{1}{2}$ " to about 1/32", and more preferably in the range of about  $\frac{1}{4}$ " to about 1/16".

The percent by weight as based upon the total weight of the manganese-containing material or composition of the manganese (calculated as MnO) is preferably in the range of about 35% to 99% by weight, and more preferably about 50% to 95% by weight.

A preferred method for reducing the sulfur content (calculated as elemental sulfur) of a hydrocarbon material into a range of about 0.1 to about 10 ppm. is a process hydrotreating or hydrofining. Hydrocarbon hydrotreating or hydrofining, as defined herein means a process wherein a hydrocarbon material containing an undesirable contaminant, e.g. sulfur or nitrogen, is contacted with a catalyst in the presence of hydrogen (H<sub>2</sub>) at conditions to form compounds, e.g. H<sub>2</sub>S and NH<sub>3</sub>, of the undesirable contaminants which can be removed from the hydrocarbon material by conventional means, e.g. simple distillation.

Examples of catalysts employed in hydrofining are comprised of composites of Group VIB or Group VIII metal hydrogenating (hydrogen transfer) components, or both, with an inorganic oxide base, or support, typically alumina. Typical catalysts are molybdena or alumina, cobalt molybdate on alumina, nickel molybdate on alumina or nickel tungstate. The specific catalyst used depends on the particular application. Cobalt molybdate catalyst is often used when sulfur removal is the primary interest. The nickel catalysts find application in the treating of cracked feedstocks for olefin or aromatic saturation. Sweetening (removal of mercaptans) is a preferred application for molybdena catalysts.

Three basic types of hydrocarbon reactions occur during hydrofining; a first which involves removal of sulfur by hydrodesulfurization (sulfur being eliminated in the form of hydrogen sulfide), a second which involves the removal of oxygen to improve stability and combustion characteristics, and a third involving the saturation of olefins and aromatic compounds with hydrogen. As to the first type, essentially four types of sulfur containing compounds, i.e., mercaptans, disul-

fides, thiophenes and benzothiophenes, are involved in the hydrodesulfurization reactions. The mercaptans and disulfide types are representative of a high percentage of the total sulfur found in the lighter virgin oils, such as virgin naphtha and heating oil. The thiophenes and benzothiophenes generally appear as the predominant sulfur form in heavy virgin oils and in cracked stocks of all boiling ranges. In the type of reaction involving oxygen removal, hydrogen reacts with oxygen compounds; condensation of the hydroxyl groups with hydrogen forms water. The removal of oxygen provides stable and clean burning fuels, and the hydrofinates are generally free of oxygen compounds.

Suitable desulfurization conditions useful in this invention include a quantity of catalyst, preferably disposed in one or more fixed-bed reaction zones, such that the liquid hourly space velocity (defined as volumes of fresh feed charge per hour per volume of catalyst disposed within the zone) is preferably within the range from about 0.4 to about 10.0. In general, lower space velocities are utilized with higher boiling, more severely contaminated feedstocks, while higher space velocities are utilized with feedstocks which are not severely contaminated. Hydrogen circulation through the catalyst bed, during processing, is a preferred technique from the standpoint of maintaining a "clean" catalytic composite, or one in which the deactivation rate due to the deposition of carbonaceous material is inhibited. Hydrogen circulation rates ranging from about 450 to about 15,000 standard cubic feet per barrel (scf/b), preferably about 500 to about 3000 scf/b are utilized, depending primarily on the character of the feedstock material and the desired results. Operating pressures will generally range from about 150 to about 5,000 psig, preferably about 200 to 750 psig while the catalyst bed inlet temperature is generally maintained in the range from about 200° to about 800° F. (93° to 425° C.), preferably about 400° to 700° F. (205° to 370° C.). Since the reactions being effected are exothermic in nature, a temperature increase will be experienced as the feedstock flows through the catalyst bed resulting in a higher catalyst bed outlet temperature. A preferred technique limits the temperature increase to about 100° F. (38° C.), and sometimes even about 250° F. (121° C.). Conventional quench streams introduced at intermediate locations in the catalyst bed can be used to control bed temperatures.

In order to significantly reduce the sulfur content of a hydrocarbon material in the presence of H<sub>2</sub>, the preferred process conditions within a zone containing a manganese-containing material as reactant are: temperature in the range of about 600° to 1000° F. (315° to 538° C.), more preferably about 650° to 850° F. (343° to 454° C.), a pressure in the range of about 150 to 750 psig and preferably 150 to 700 psig, a hydrogen/hydrocarbon mole ratio in the range of about 1/1 to 30/1 and a space velocity in the range of about 500 to 50,000 volume of gas/hour/volume of reactant.

In order to significantly reduce the sulfur content of a hydrocarbon material in the substantial absence of H<sub>2</sub>, e.g. when the amount of H<sub>2</sub> present in the hydrocarbon material is less than about 2% by weight of that hydrocarbon material, the preferred process conditions within a zone containing a manganese-containing material as reactant are: temperatures in the range of about 500° to 1000° F. (260° to 538° C.), more preferably, about 650° to 850° F. (343° to 454° C.), a pressure in the range of about 50 to 750 psig, and preferably 150 to 700

psig., and a space velocity in the range of about 500 to 50,000 volume of gas/hour/volume of reactant.

The reforming catalyst useful in the present invention comprises a solid porous support, e.g., alumina, at least one platinum-group metal component and preferably at least one halogen component. It is preferred that the solid porous support be a material comprising a major amount of alumina having a surface area of about 25 m.<sup>2</sup>/gm. to about 600 m.<sup>2</sup>/gm. or more. The solid porous support comprises a major proportion, preferably at least about 80%, and more preferably at least about 90%, by weight of the catalyst. The preferred catalyst support, or base, is an alumina derived from hydrous alumina predominating in alumina trihydrate, alumina monohydrate, amorphous hydrous alumina and mixtures thereof; more preferably, alumina monohydrate, amorphous hydrous alumina and mixtures thereof, which alumina when formed as pellets and calcined, has an apparent bulk density of about 0.60 gm./cc. to about 0.85 gm./cc., pore volume of about 0.45 cc./gm. to about 0.70 cc./gm., and surface area of about 100 m.<sup>2</sup>/gm. to about 500 m.<sup>2</sup>/gm. The solid porous support may contain, in addition, minor proportions of other well known refractory inorganic oxides such as silica, zirconia, magnesia and the like. However, the most preferred support is substantially pure alumina derived from hydrous alumina predominating in alumina monohydrate, amorphous hydrous alumina and mixtures thereof.

The alumina support may be synthetically prepared in any suitable manner and may be activated prior to use by one or more treatments including drying, calcination, steaming and the like. Thus, for instance, hydrated alumina in the form of a hydrogel can be precipitated from an aqueous solution of a soluble aluminum salt such as aluminum chloride. Ammonium hydroxide is a useful agent for effecting the precipitation. Control of the pH to maintain it within the values of about 7 to about 10 during the precipitation is desirable for obtaining a good rate of conversion. Extraneous ions, such as halide ions, which are introduced in preparing the hydrogel, can, if desired, be removed by filtering the alumina hydrogel from its mother liquor and washing the filter cake with water. Also, if desired, the hydrogel can be aged, say for a period of several days. The effect of such aging is to build up the concentration of alumina trihydrate in the hydrogel. Such trihydrate formation can also be enhanced by seeding an aqueous slurry of the hydrogel with alumina trihydrate crystallites, for example, gibbsite.

The alumina may be formed into macrosize particles of any desired shape such as pills, cakes, extrudates, powders, granules, spheres, and the like using conventional methods. The size selected for the macrosize particles can be dependent upon the intended environment in which the final catalyst is to be used—as, for example, whether in a fixed or moving bed reaction system. Thus, for example, where as in the preferred embodiment of the present invention, the final catalyst is designed for use in hydrocarbon reforming operations employing a fixed bed of catalyst, the alumina will preferably be formed into particles having a minimum dimension of at least about 0.01 inch and a maximum dimension up to about one-half inch or one inch or more. Spherical particles having a diameter of about 0.03 inch to about 0.25 inch, preferably about 0.03 inch to about 0.15 inch, are often useful, especially in a moving bed reforming operation.

As indicated above, the catalyst utilized in the present invention also contains a platinum-group metal. The platinum-group metals include platinum, palladium, rhodium, iridium, ruthenium, osmium and the like with platinum being preferred for use in the present invention. The platinum-group metal, such as platinum, may exist within the final catalyst at least in part as a compound such as an oxide, sulfide, halide and the like, or in the elemental state. The platinum-group metal component preferably comprises about 0.01% to about 3.0%, more preferably about 0.05% to about 1.0%, by weight of the catalyst, calculated in an elemental state. Excellent results are obtained when the catalyst contains about 0.2% to about 0.9% by weight of the platinum-group metal component.

The platinum group component may be incorporated in the catalyst in any suitable manner, such as by coprecipitation or cogellation with the alumina support, ion-exchange with the alumina support and/or alumina hydrogel, or by the impregnation or the alumina support and/or alumina hydrogel at any stage in its preparation and either after or before calcination of the alumina hydrogel. One preferred method for adding the platinum-group metal to the alumina support involves the utilization of a water soluble compound of the platinum-group metal to impregnate the alumina support prior to calcination. For example, platinum may be added to the support by comingling the uncalcined alumina with an aqueous solution of chloroplatinic acid. Other water-soluble compounds of platinum may be employed as impregnation solutions, including, for example, ammonium chloroplatinate and platinum chloride. The utilization of a platinum-chlorine compound, such as chloroplatinic acid, is preferred since it facilitates the incorporation of both the platinum and at least a minor quantity of the halogen component of the catalyst, described hereinafter. It is preferred to impregnate the support with the platinum-group metal when it, the support, is in a hydrous state. Following this impregnation, the resulting impregnated support is shaped (e.g., extruded), dried and subjected to a high temperature calcination or oxidation procedure at a temperature in the range of about 700° F. to about 1500° F. (370° to 815° C.), preferably of about 850° F. to about 1300° F. (454° to 704° C.), for a period of time of about one hour to about 20 hours, preferably of about one hour to about five hours. The major portion of the halogen component can be added to this otherwise fully composited calcined catalyst by contacting this catalyst with a substantially anhydrous stream of halogen-containing gas.

An optional and preferred constituent of the catalyst utilized in the present invention is an additional component exemplified by rhenium. This component may be present as an elemental metal, as a chemical compound, such as the oxide, sulfide, or halide, or in a physical or chemical association with the alumina support and/or the other components of the catalyst. Generally, the rhenium is utilized in an amount which results in a catalyst containing about 0.01% to about 5%, preferably about 0.05% to about 1.0%, by weight of rhenium, calculated as the elemental metal. The rhenium component may be incorporated in the catalyst in any suitable manner and at any stage in the preparation of the catalyst. The procedure for incorporating the rhenium component may involve the impregnation of the alumina support or its precursor either before, during or after the time the other components referred to above are added. The impregnation solution can in some cases be

an aqueous solution of a suitable rhenium salt such as ammonium perrhenate, and the like salts or it may be an aqueous solution of perrhenic acid. In addition, aqueous solutions of rhenium halides such as the chloride may be used if desired. It is preferred to use perrhenic acid as the source of rhenium for the catalysts utilized in the present invention. In general, the rhenium component can be impregnated either prior to, simultaneously with, or after the platinum-group metal component is added to the support. However, it has been found that good results are achieved when the rhenium component is impregnated simultaneously with the platinum-group component. In the instance where the catalyst support, e.g. alumina derived from hydrous alumina predominating in alumina monohydrate is formed into spheres using the conventional oil drop method, it is preferred to add the platinum-group metal and rhenium after calcination of the spheroidal particles. The presently useful catalyst may include a minor, catalytically effective amount of one or more other well known promoters, such as germanium, tin, gold, cadmium, lead, the rare earth metals, and mixtures thereof.

Another optional and preferred constituent of the catalyst used in the present invention is a halogen component. Although the precise chemistry of the association of the halogen component with the alumina support is not entirely known, it is customary in the art to refer to the halogen component as being combined with the alumina support, or with the other ingredients of the catalyst. This combined halogen may be fluorine, chlorine, bromine, and mixtures thereof. Of these, fluorine and, particularly, chlorine are preferred for the purposes of the present invention. The halogen may be added to the alumina support in any suitable manner, either during preparation of the support, or before or after the addition of the catalytically active metallic component or components. For example, at least a portion of the halogen may be added at any stage of the preparation of the support, or to the calcined catalyst support, as an aqueous solution of an acid such as hydrogen fluoride, hydrogen chloride, hydrogen bromide and the like or as a substantially anhydrous gaseous stream of these halogen-containing components. The halogen component, or a portion thereof, may be composited with alumina during the impregnation of the latter with the platinum-group component and/or rhenium component; for example, through the utilization of a mixture of chloroplatinic acid and/or perrhenic acid and hydrogen chloride. In another situation, the alumina hydrogel which is typically utilized to form the alumina component may contain halogen and thus, contribute at least a portion of the halogen component to the final composition or composite. For purposes of the present invention, when the catalyst support is used in the form of an extrudate, the major portion of the halogen component can be added to the otherwise fully composited calcined catalyst by contacting this catalyst with a stream of halogen-containing gas. When the catalyst is prepared by impregnating calcined, formed alumina, for example, spheres produced by the conventional oil drop method, it is preferred to impregnate the support simultaneously with the platinum-group metal, rhenium component and halogen. In any event, the halogen is preferably added in such a manner as to result in a fully composited catalyst that contains about 0.1% to about 5% and preferably about 0.2% to about 1.5% by weight of halogen calculated on an elemental basis.

The final fully composited catalyst prepared, for example, by a method set forth above, is generally dried at a temperature of about 200° F. (93° C.) to about 600° F. (315° C.) for a period of about 2 to about 24 hours or more and finally calcined at a temperature of about 700° F. (370° C.) to about 1500° F. (815° C.) preferably about 850° F. (454° C.) to about 1300° F. (704° C.) for a period of about  $\frac{1}{4}$  hour to about 20 hours and preferably about  $\frac{1}{4}$  hour to about 5 hours.

10 The resultant calcined catalyst may be subjected to reduction prior to use in reforming hydrocarbons. This step is designed to insure chemical reduction of at least a portion of the metallic components.

15 The reducing media may be contacted with the calcined catalyst at a temperature of about 800° F. (427° C.) to about 1200° F. (649° C.) and at a pressure in the range of about 0 psig. to about 500 psig. and for period of time of about 0.5 to about 10 hours or more and, in any event, for a time which is effective to chemically 20 reduce at least a portion, preferably a major portion, of each of the metallic components, e.g., platinum-group metal and rhenium component, of the catalyst. By chemical reduction is meant the lowering of oxidation states of the metallic components below the oxidation 25 state of the metallic components in the unreduced catalyst. For example, the unreduced catalyst may contain platinum salts in which the platinum has an oxidation state which can be lowered or even reduced to elemental platinum by contacting the unreduced catalyst with 30 hydrogen. This reduction treatment is preferably performed in situ, (i.e., in the reaction zone in which it is to be used), as part of a start-up operation using fresh unreduced catalyst or regenerated (e.g., regenerated by treatment with an oxygen-containing gas stream) catalyst. The process of the present invention may be practiced using virgin catalyst and/or catalyst that has previously been used to reform hydrocarbon and has been 35 subsequently subjected to conventional treatments to restore, e.g., regenerate and/or reactivate, the hydrocarbon reforming activity and stability of the catalyst.

40 Hydrocarbon reforming conditions often include a hydrogen to hydrocarbon mole ratio in the range of about 1/1 to about 30/1, preferably about 2/1 to about 20/1; reaction pressure in the range of about 50 psig to about 1000 psig, preferably about 100 psig to about 600 psig and more preferably about 200 psig to about 400 psig; and a weight hourly space velocity, i.e., (whsv) in the range of about 0.5 to about 10.0 or more, preferably about 1.5 to about 6.0.

45 For optimum reforming results, the temperature in the reaction zone should preferably be within the range of about 700° F. (370° C.) to about 1100° F. (593° C.), more preferably in the range of about 800° F. (427° C.) to about 1050° F. (565° C.). The initial selection of the temperature within the broad range is made primarily as a function of the desired octane of the product reformatte, considering the characteristics of the charge stock and of the catalyst. The temperature may be slowly increased during the run to compensate for the inevitable deactivation that occurs, to provide a constant octane product.

50 The content of halide on the reforming catalyst is 55 preferably maintained throughout the reforming process in order to maintain the activity of the reforming catalyst. As the content of the halide on the catalyst decreases, the activity of the catalyst also tends to decrease. Optionally, halogen components are added to the reforming zone either with the feedstock and/or

with the hydrogen ( $H_2$ ) so as to maintain the halogen component content on the catalyst. Halide-containing compounds which are added to the reforming zone preferably are or break down into hydrogen halide gas which readily reacts with the reforming catalyst so as to maintain the halide content at an optimal level for the catalyst. The addition of halide-containing compounds can result in the gas comprising hydrogen ( $H_2$ ) and other volatile components in the recycle line containing a concentration of volatile halide compounds, e.g. hydrogen halide. The concentration in moles of volatile halide compounds to total moles of the gas is up to about 10 ppm., preferably up to about 5 ppm., and more preferably at least about 0.01 ppm. Preferably this concentration is in the range of between about 0.05 to about 1 ppm. Examples of compounds which may be added to the reforming zone either continuously with the reforming of hydrocarbon material or in the absence of hydrocarbon material are volatile hydrocarbon halides such as carbon tetrachloride, chloroform and the like.

#### BRIEF DESCRIPTION OF THE DRAWINGS

FIG. 1 is a schematic flow diagram of a reforming process employing both a hydrodesulfurization zone and a zone for trapping or absorbing hydrogen sulfide.

FIG. 2 is a system for reforming naphtha feedstocks.

FIG. 3 is a graph showing the relative performance of sulfur traps employing  $MnO$ ,  $CuCr$ , HDS-20A, and  $Ni$  on Kieselguhr.

FIG. 4 is a graph showing how breakthrough times are determined in Example 4.

FIG. 5 is a graph showing sulfur removal as a function of sulfur removal zone temperature.

#### DETAILED DESCRIPTION OF THE DRAWINGS

The flow diagram of FIG. 1 comprises transfer lines 51, 53, 55, 57, 59, 71, 75 and 80, a hydrodesulfurization zone 52, a zone 54 for removing or absorbing hydrogen sulfide gas and a reforming zone 56.

A naphtha feedstock enters hydrodesulfurization zone 52 via transfer line 51. Leaving hydrodesulfurization zone 52 via one or more transfer lines collectively represented by transfer line 55 are volatiles comprising, for example, low molecular weight hydrocarbons, hydrogen sulfide, ammonia and hydrogen. A hydrogen makeup line 53 transfers hydrogen into zone 52. A portion of this hydrogen may be taken from recycle line 71. The possibility of drawing some of this hydrogen from the recycle line is indicated by the dotted line 80. Hydrodesulfurized hydrocarbon feedstock is transferred from zone 52 to zone 54 where at least a portion of the residual hydrogen sulfide is removed by contact with a manganese-containing composition comprising, for example, an oxide of manganese. The hydrocarbon feedstock, having been treated by contact with an oxide of manganese, preferably manganese oxide, is then transferred via line 59 to reformer 56. Leaving reformer 56 via line 75 is the reformed product. Transferred through recycle line 71 from reformer 56 to sulfur trap zone 54 is a recycle gas comprising primarily hydrogen and volatile hydrocarbons, wherein the ratio in moles of hydrogen/hydrocarbon is in the range about 1/1 to 30/1, and preferably about 2/1 to 20/1.

FIG. 2 discloses a system for reforming hydrocarbon materials comprising a hydrodesulfurization zone 2, a heat exchanger 4, a zone 6 for absorbing or removing hydrogen sulfide (sulfur trap), a furnace 8, a reformer

10, a separator 12, a compressor 14, and transfer lines 19, 21, 22, 23, 25, 27, 29, 31, 33, 35, 37, 39, 41, 43, and 45, and valves 48. Alternate locations for sulfur traps are indicated at locations A, B, C, D, E, and F. A liquid phase sulfur trap zone at location E can be located prior to the junction of transfer lines 41 and 23 or after F. The percent by weight of hydrogen ( $H_2$ ) at location E is less than about 2% by weight based on hydrocarbon material also present at this location. Additional  $H_2$  can be added through transfer line 22 as required. With a liquid phase sulfur trap zone at E, there is in effect no recycle gas except possibly from zone 2 and the temperatures within zones at E and F being prior to heat exchanger 4 are such as to maintain a liquid phase therein of a hydrocarbon material.

Hydrocarbon feedstock, e.g. straight-run, catalytically cracked, or thermally cracked naphthas, or any other naphtha fraction suitable for octane value improvement, boiling up to about 450° F. (232° C.) enters via line 19 into a hydrodesulfurization zone 2 where the feedstock is hydrotreated and organic sulfur is converted to hydrogen sulfide. Make-up hydrogen enters zone 2 via line 45. An optional take-off line from recycle line 41 can be tied indirectly into 45 as indicated by dotted line 43 to make use of a net excess of hydrogen produced in reformer 10.

Depending upon the severity of the hydrodesulfurization treatment, nitrogen compounds can also be hydrogenated to produce ammonia.

Leaving hydrodesulfurization zone 2 by means of one or more transfer lines collectively represented by transfer line 21 are volatiles comprising, for example, low molecular weight hydrocarbons, hydrogen sulfide, ammonia and hydrogen. Separation by means of transfer line 21 is achieved based on physical differences, e.g. vapor pressures or boiling points. Such separation based on physical properties is to be distinguished from separations based on chemical or physical interactions such as occurs in zone 6 or other sulfur removal zones optionally located at A, B, C, D, E or F.

A variety of hydrodesulfurization catalysts can be used, which includes a combination of oxides of elements from Group 8 and Group 6b supported on a support, e.g., alumina.

Process conditions within the hydrodesulfurization reactor (not shown) but which is part of the hydrodesulfurization zone 2 schematically represented as a box involve temperatures in the range of about 200° F. (93° C.) to about 800° F. (427° C.), preferably in the range of about 400° F. (205° C.) to about 700° F. (370° C.), pressure in the range 150 psig to about 5000 psig preferably about 200 to about 750 psig, hydrogen concentration in the range of about 450 scf/b to about 15,000 scf/b, preferably about 500 to 3000 scf/b, and a liquid hourly space velocity in the range of about 0.4 to about 10.

Hydrotreated material or stripper bottoms containing a significantly reduced concentration of sulfur, e.g., about 2 to about 20 ppm, is transferred in line 23 through a heat exchanger 4. The temperature of the hydrotreated material is raised to between about 550° F. (288° C.) and about 850° F. (455° C.) at a pressure of from about 150 to about 750 psig. Heated material passes via line 25 through valve 48 into line 27, then, optionally, through zone 6 containing a supported manganese oxide and via line 29 through another valve 48 into transfer line 31. The arrangement of valves 48 permits a bypass of sulfur trap 6.

The heated material passing via line 31 is further heated in furnace 8 to a temperature in the range of about 850° F. (455° C.) to about 950° F. (510° C.).

The heated material from furnace 8 optionally can pass through a sulfur trap at location A and then into reformer 10.

In reformer 10, the heated hydrocarbon material is contacted with a typical reformer catalyst, e.g., a platinum-group metal catalyst preferably having a halide component and either with or without rhodium, at reforming conditions, such as a temperature in the range 650° F. (353° C.) to about 1050° F. (565° C.), a pressure in the range of about 5 psig to about 600 psig, a hydrogen/hydrocarbon mole ratio of about 1/1 to 30/1, and a space velocity in the range of about 0.5 to about 15

10. Ordinarily, two or more reforming zones with heaters therebetween in series are employed.

The reformed product produced in reformer 10 is transferred through line 35 to a separator 12. Separator 12 separates a liquid hydrocarbon product and a volatile product consisting of hydrogen and volatile hydrocarbons. The hydrogen and other volatiles, e.g., low molecular weight hydrocarbons, are removed through line 39 then into recycle line 41. Optionally, a portion of the volatiles can be passed through a sulfur trap at location C prior to entering line 41. A compressor 14 is located on line 41 to pressurize and transfer volatile components from line 39. The mole ratio of H<sub>2</sub>/HC (hydrocarbon) in recycle line 41 is in the range of about 1/1 to about 30/1. Reformed liquid product exits through line 37.

In reformer 10, there is a reforming catalyst which contains a platinum-group metal component and a halogen component. The halogen component is replenished during the reforming cycle by adding volatile halides to the hydrocarbon material entering line 19. Optionally, volatile halides can be introduced into the H<sub>2</sub> make up line 3, 22 or 45 or the recycle line 41. The concentration in moles of hydrohalide, e.g., HCl, per total moles of gas in recycle line 41 is in the range of about 0.05 to about 1 ppm. In any event, halides are preferably added either on a continuous or intermittent basis so as to maintain the halide content of the reforming catalyst.

A significant advantage of the process of this invention over that disclosed in U.S. Pat. No. 3,898,153 (1975) cited hereinbefore is the fact that there is no need to precede each sulfur trap of this invention with a trap or scavenging zone for volatile halides, e.g. chlorides.

#### EXAMPLE 1

The following thermodynamic calculations compare zinc oxide and manganous oxide and with EXAMPLES 3 and 4 establish that:

(1) Formation of metal sulfides from the oxides of both manganese and zinc is very favorable in the presence of hydrogen sulfide gas;

(2) The formation of zinc chloride from zinc oxide by reaction with hydrochloric acid gas is less thermodynamically favored than the formation of manganous chloride from manganous oxide. However, as a reactant, both manganous chloride and zinc chloride are not thermodynamically favored under the following conditions: temperature in the range 650° to 1000° F. (343° to 538° C.), an H<sub>2</sub>O/Cl mole ratio in recycle gas of 20/1 to 60/1, a recycle mole ratio of H<sub>2</sub>/HC in the range 3/1 to 30/1, a pressure in the range 150-750 psig and a space velocity in the range 500 to 50,000 vol. of gas/hr./vol.

60

65 of reactant.

(3) Conversion of the metal sulfide to the metal chloride in hydrogen sulfide gas by hydrochloric gas is less favorable with zinc sulfide than with manganous sulfide. The equilibrium data of Table 1 establishes this point.

In the CRC Handbook of Chemistry of Physics, Forty-Seventh Edition, 1966-1967, and the Bureau of Mines, Report of Investigations 5600, Thermodynamics Properties of Manganese and its Compounds by Alla D. Mah, there is reported that both zinc chloride and zinc metal have vapor pressures which are much higher than manganous chloride and are therefore expected to tend to migrate more quickly from a sulfur trap to a zone containing reforming catalyst upon the formation of any chlorides.

TABLE 1

H<sub>2</sub>S FROM MnS AND ZnS BY THE ACTION OF HCl AT HOUSTON 733 GUARD REACTOR CONDITIONS



| M =<br>Temp., °F. | Manganese            |                      | Zinc                 |                      |
|-------------------|----------------------|----------------------|----------------------|----------------------|
|                   | 440                  | 620                  | 800                  | 980                  |
| 25                | $1.7 \times 10^{-1}$ | $1.0 \times 10^{-2}$ | $1.9 \times 10^{-5}$ | $3.8 \times 10^{-7}$ |
| 30                | $2.2 \times 10^{-3}$ | $9.7 \times 10^{-5}$ | $9.3 \times 10^{-6}$ | $1.4 \times 10^{-8}$ |

Equilibria and Calculations



The following equilibrium constants were calculated from an expression which relates K<sub>e</sub> to temperature.

| °F. | °K.                          |
|-----|------------------------------|
| 440 | $500 \quad 6.76 \times 10^5$ |
| 620 | $600 \quad 3.31 \times 10^3$ |
| 800 | $700 \quad 7.41 \times 10^1$ |
| 980 | $800 \quad 4.29 \times 10^0$ |

Source: Kitchener, J.A., Ignatowicz, S., Trans. Faraday Soc. 47,1278, (1951).

$$\log_{10} K' = \log_{10} (P^2_{\text{HCl}} / P_{\text{H}_2\text{O}}) = -\frac{6.930}{T} + 8.03$$

p = atm

T = °K.

K' = reverse of reaction A

$$\log_{10} K' = -\log_{10} K$$

The K<sub>e</sub> values listed above were used to calculate the HCl<sub>actual</sub>/HCl<sub>equil</sub> numbers for zinc shown below.

| Temp., °F. | H <sub>2</sub> O/Cl | HCl <sub>actual</sub> /HCl <sub>equil</sub> |                            |
|------------|---------------------|---------------------------------------------|----------------------------|
|            |                     | at 10 ppm H <sub>2</sub> O                  | at 20 ppm H <sub>2</sub> O |
| 50         | 5                   | 2.34 E-1                                    | 3.02 E0                    |
|            | 15                  | 7.83 E-2                                    | 1.10 E-1                   |
|            | 30                  | 3.91 E-2                                    | 5.53 E-2                   |
|            | 100                 | 1.17 E-2                                    | 1.66 E-2                   |
| 700        | 5                   | 7.22 E-2                                    | 1.02 E-1                   |
|            | 15                  | 2.41 E-2                                    | 3.40 E-2                   |
|            | 30                  | 1.20 E-2                                    | 1.71 E-2                   |
|            | 100                 | 3.60 E-3                                    | 5.11 E-3                   |
| 800        | 5                   | 2.72 E-2                                    | 3.83 E-2                   |
|            | 15                  | 9.07 E-3                                    | 1.28 E-2                   |
|            | 30                  | 4.52 E-3                                    | 6.41 E-3                   |
|            | 100                 | 1.36 E-3                                    | 1.92 E-3                   |

Total pressure was 350 psig.

Equilibria and Calculations



Equilibrium Constants\*

| °K  | K <sub>Equil</sub> |
|-----|--------------------|
| 500 | $2.90 \times 10^9$ |
| 600 | $6.21 \times 10^6$ |
| 700 | $7.98 \times 10^4$ |
| 800 | $3.14 \times 10^3$ |

Equilibrium Constants, °F., Interpolated\*\*

TABLE 1-continued

| °F. | K <sub>Equil</sub>     |
|-----|------------------------|
| 600 | 1.25 × 10 <sup>7</sup> |
| 650 | 3.04 × 10 <sup>6</sup> |
| 700 | 8.40 × 10 <sup>5</sup> |
| 750 | 2.58 × 10 <sup>5</sup> |
| 800 | 8.68 × 10 <sup>4</sup> |
| 850 | 3.18 × 10 <sup>4</sup> |
| 900 | 1.26 × 10 <sup>4</sup> |

\*See Page 21 Bureau of Mines, Report of Investigations 5600, entitled Thermodynamic Properties of Manganese and Its Compounds, by Alla D. Mah

\*\*Interpolated using a linear fit of log K vs. 1/T.

| Temp., °F. | H <sub>2</sub> O/Cl | HCl <sub>actual</sub> /HCl <sub>equil</sub> |                            |
|------------|---------------------|---------------------------------------------|----------------------------|
|            |                     | at 10 ppm H <sub>2</sub> O                  | at 20 ppm H <sub>2</sub> O |
| 600        | 5                   | 1.11 E1                                     | 1.57 E1                    |
|            | 15                  | 3.71 E0                                     | 5.24 E0                    |
|            | 30                  | 1.85 E0                                     | 2.63 E0                    |
|            | 100                 | 5.54 E-1                                    | 7.86 E-1                   |
|            | 5                   | 5.50 E0                                     | 7.76 E0                    |
|            | 15                  | 1.84 E0                                     | 2.59 E0                    |
| 650        | 30                  | 9.17 E-1                                    | 1.30 E0                    |
|            | 100                 | 2.75 E-1                                    | 3.88 E-1                   |
|            | 5                   | 2.89 E0                                     | 4.09 E0                    |
|            | 15                  | 9.65 E-1                                    | 1.36 E0                    |
|            | 30                  | 4.81 E-1                                    | 6.83 E-1                   |
|            | 100                 | 1.44 E-1                                    | 2.05 E-1                   |
| 700        | 5                   | 1.60 E0                                     | 2.26 E0                    |
|            | 15                  | 5.35 E-1                                    | 7.54 E-1                   |
|            | 30                  | 2.67 E-1                                    | 3.78 E-1                   |
|            | 100                 | 8.00 E-2                                    | 1.13 E-1                   |
|            | 5                   | 9.29 E-1                                    | 1.31 E0                    |
|            | 15                  | 3.10 E-1                                    | 4.38 E-1                   |
| 750        | 30                  | 1.55 E-1                                    | 2.20 E-1                   |
|            | 100                 | 4.64 E-2                                    | 6.57 E-2                   |
|            | 5                   | 5.63 E-1                                    | 7.94 E-1                   |
|            | 15                  | 1.88 E-1                                    | 2.65 E-1                   |
|            | 30                  | 9.38 E-2                                    | 1.33 E-1                   |
|            | 100                 | 2.81 E-2                                    | 3.98 E-2                   |

Total pressure was 350 psig.



| °K. | K <sub>eq</sub>         |
|-----|-------------------------|
| 500 | 3.69 × 10 <sup>3</sup>  |
| 600 | 6.94 × 10 <sup>0</sup>  |
| 700 | 1.36 × 10 <sup>-1</sup> |
| 800 | 5.07 × 10 <sup>-3</sup> |

\*Calculated from ΔG° values as tabulated below.

Free Energy of Formation, ΔG°, Kcal/mole

| °K.                  | 500    | 600    | 700    | 800    | Ref. |
|----------------------|--------|--------|--------|--------|------|
| ZnS                  | -39.58 | -39.17 | -38.73 | -38.26 | A    |
| HCl                  | -23.22 | -23.42 | -23.60 | -23.77 | B    |
| ZnCl <sub>2</sub> ** | -78.71 | -73.93 | -69.88 | -65.27 |      |
| H <sub>2</sub> S     | -15.47 | -14.39 | -13.27 | -12.13 | C    |
| H <sub>2</sub> O     | -52.36 | -51.15 | -49.91 | -48.64 | D    |
| ZnO                  | -71.30 | -68.95 | -66.60 | -64.05 | E    |

\*\*Since these values could not be found directly in the literature at temperatures other than 298° K. (std. state), the numbers shown are back-calculated from K<sub>eq</sub> values shown in Appendix Section A. for the ZnO + 2HCl = 3nCl<sub>2</sub> + H<sub>2</sub>O equilibrium and ΔG° values for ZnO, HCl and H<sub>2</sub>O tabulated above. These numbers are believed to be accurate because the ΔG° calculated at 298° K. (-87.8 Kcal/mole) by this method agrees well with the known value (-88.3 Kcal/mole).<sup>F</sup>

References:

- A. U.S. Bureau of Mines Bulletin 601 (Reprint of 406), p. 65-66.
- B. U.S. Bureau of Mines Bulletin 668, p. 102.
- C. U.S. Bureau of Mines Bulletin 668, p. 103.
- D. U.S. Bureau of Mines Bulletin 542, p. 22-23.
- E. U.S. Bureau of Mines Bulletin 542, p. 58.
- F. NBS Technical Note 270-3, Selected Values of Chemical Thermodynamic Properties, U.S. Dept. of Commerce.

### EXAMPLE 2

A manganous oxide sulfur trap material was prepared as follows. Manganous oxide powder, as received from Diamond Shamrock, was tabletted with 5% graphite plus 3% Sterotex (a powdered vegetable stearine sold by Capital City Products Co., Columbus, Ohio) using a Stokes tabletting machine. The  $\frac{3}{8}'' \times 3/32''$  tablets were

then calcined for three hours at 900° F. (482° C.) in a muffle furnace.

The crush strength of the above material was found to increase upon sulfiding.

### EXAMPLE 3

The relative performance as a reactant for removing at least a portion of a sulfur component from a hydrogen (H<sub>2</sub>) stream of the graphite supported manganous oxide (95% MnO/5% graphite) prepared according to Example 2, copper-chromia (CuCr) and nickel on kieselguhr are shown in FIG. 3. The processing conditions employed were 500 psig, 25000 SCF GAS/Hr/Ft<sup>3</sup>

BED (60° F., 1 ATM), and nominally 2 ppm. H<sub>2</sub>S in plant H<sub>2</sub> as feedstock for about one week. In all tests, exit gas concentrations were less than 0.01 ppm. H<sub>2</sub>S. The MnO was tested at 650° F. (343° C.). The copper chromia and nickel compositions were tested at 200° F. (93° C.) because they are suited only for recycle gas service.

HDS-20 is a cobalt-molybdenum trilobar catalyst, which is a material sold by American Cyanamid.

The 55% by weight of nickel on kieselguhr is a commercially available material sold by Harshaw Chemical Company, a Division of Kewanee Oil Co. of Cleveland, Ohio.

The copper-chromia material can be made according to methods disclosed in U.S. Pat. No. 4,049,842 (1977). The use here of this material is different from that disclosed in the patent.

The percent by weight of sulfur within the reactant was determined for each of ten equal segments along the length of a packed bed of a one-inch down flow standard reactor. A graph, beginning at the up-stream end, plotting the weight percent of sulfur in each of ten equal segments along the length of the down-stream reactor versus the corresponding segment is plotted in FIG. 3.

A significantly superior performance of manganous oxide is clear from the fact that the time at which significant amounts, e.g., greater than 1 ppm of hydrogen sulfide gas will leak through the sulfur trap material or reactant will occur last for the manganous oxide as compared to all others. This is shown by the approximation discussed in the following example.

### EXAMPLE 4

An estimate of the time that hydrogen sulfide gas will break through a packed reactor in the case of zinc oxide versus manganous oxide is as follows: Referring to FIG. 4, a bed profile is experimentally determined wherein the percent by weight of sulfur loading is represented by an Area A. If breakthrough was not actually observed experimentally, the curve with Area B is approximated by moving the leading edge of the experimentally determined bed profile to the right until breakthrough would be expected to occur. A tangent is then taken at a point on the leading portion of this profile at expected breakthrough and extrapolated back to a reasonable loading of sulfur in percent by weight for segment 1 of the packed bed. In the case of manganous oxide, the maximum loading in percent by weight of segment 1 of the packed material was determined to be approximately midway between the percent by weight determined experimentally, and the maximum percent by weight theoretically obtainable at equilibrium. Of course, a variety of extrapolations are possible depending upon the point on the leading edge of the curve

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

selected. Values greater than the percent by weight at equilibrium are clearly unreasonable and were rejected.

An estimate of the amount of sulfur within the total bed at the moment of breakthrough is the area under the curve for Area B approximated as above. The length of time it would take to pass that amount of sulfur through the bed under the processing conditions of the test yields an estimate of the breakthrough time.

Based on this method of approximation, a loading in weight percent of sulfur at breakthrough for manganous oxide was estimated to be 17% to 20%. A supplier of zinc oxide reported that the loading in weight percent of sulfur at breakthrough for zinc oxide was 3% under equivalent packing and operation conditions. The relative breakthrough time for these materials assuming equal packing weights, is directly proportional to the ratio of sulfur loadings for each at breakthrough. Therefore, the breakthrough time of manganous oxide is about 5.5 to 6.6 times that for zinc oxide.

#### EXAMPLE 5

In order to determine the consequence of adding either zinc oxide or manganous oxide to a reforming catalyst with regard to both activity and stability, the following test was run. An isothermal down flow one-inch reactor was filled with 20" of catalyst diluted with an inert material of tabular nonporous, neutral, alpha-alumina. A regulated flow of hydrogen and hydrocarbon (source of hydrocarbon Midcontinent Naphtha) was maintained at test conditions by a liquid level release and a pressure control. The test conditions employed were an isothermal temperature of 950° F. (510° C.) which is approximately 28°-50° F. (15°-28° C.) higher than normal, 300 psig, 3 moles of hydrogen per mole of hydrocarbon, a space velocity of 4 grams of hydrocarbon/hour/gram of catalyst and 20 grams of catalyst charged with a pseudolog dilution in five sections. The test length was 300 hours.

A linear fit was applied to averaged raw data so that the initial value for such averaged raw data is 100 Research Octane Number Clear (RONC) at time zero; then the average slope for the first one hundred hours is a measure of the average aging rate of the particular catalyst tested.

#### SUMMARY OF RESULTS

|             | Sulfur Trap Matl.        | RONC         | Del. RONC*/<br>100 HRS.     |
|-------------|--------------------------|--------------|-----------------------------|
| A (Virgin)  | —                        | 99.6 ± .5    | -1.9 ± 0.2                  |
| B (Regen)** | MnO(10%)                 | 101.5 ± .5   | -5.1 ± 0.5                  |
| A (Virgin)  | MnO(.05%)                | 102.2 ± .5   | -1.9 ± 0.2                  |
| A (Virgin)  | MnCl <sub>2</sub> (.36%) | 101.5 ± .5   | -2.1 ± 0.2                  |
| B (Regen)** | ZnO(10%)                 | Less than 80 | Catalyst Dead, Test Aborted |

\*Corrected to 100 RONC at zero time, and Del means delta for change in RONC.  
\*\*Regen means a regenerated and a reactivated catalyst both which had previously been used to reform a Midcontinent Naphtha feedstock and to which about 10% by weight, as based on the catalyst, of powdered sulfur trap material had been added.

Two different reforming catalysts A (a platinum-rhenium catalyst) and B (a platinum catalyst) were employed. The impact on both activity and stability clearly indicates that in the case of zinc, the catalyst for all intents and purposes is ruined, whereas in the case of manganous oxide or manganous chloride, the catalyst is not adversely affected within experimental error.

The foregoing examples of this invention are intended to be illustrative only. Variations on the specific embodiments and examples disclosed would be obvious to a person of skill in the art based upon the teachings in

this specification. Such variations are intended to be within the scope of this invention.

#### EXAMPLE 6

The following liquid phase sulfur removal zones were run to compare the performance of manganese oxide versus zinc oxide.

A stream of naphtha saturated with hydrogen sulfide gas at one atmosphere and at 75° F. was passed through 10 a liquid phase sulfur removal zone consisting of either manganese oxide or zinc oxide. A sulfur analysis in part per million on the feed and end product were carried out in a semi-quantitative fashion to determine the efficiency of sulfur removal at temperatures 200°, 400°, and 15 500° F. The results are given in the following table.

#### LIQUID PHASE SULFUR TRAP TEST CONDITIONS

| 20                               | Temp | Manganese Oxide |         | ZnO  |         |
|----------------------------------|------|-----------------|---------|------|---------|
|                                  |      | Feed            | Product | Feed | Product |
| H <sub>2</sub> S/H <sub>2</sub>  | 200° | 11              | 10      | 23   | 25      |
| Saturated                        |      | 8               | 4       | —    | —       |
| Naphtha                          | 400° | 9               | 5       | 31   | 27      |
|                                  |      | 4               | 3       | 22   | 1       |
|                                  | 500° | 13              | 5       | 22   | 1       |
|                                  |      | 5               | 0       | 23   | 1       |
|                                  |      | —               | 0       | —    | —       |
| 50 ppm S as Thiophene in Naphtha | 200° | —               | —       | 43   | 40      |
|                                  | —    | —               | —       | 47   | 45      |
|                                  | 300° | 45              | —       | —    | —       |
|                                  | 47   | —               | —       | —    | —       |
|                                  | 400° | 47              | 49      | 48   | 43      |
|                                  |      | 48              | 45      | 52   | —       |
|                                  | 500° | 50              | 46      | 47   | 47      |
|                                  |      | 48              | 45      | 49   | 47      |
| 50 ppm S mercaptan in Naphtha    | 200° | —               | 46      | —    | —       |
|                                  | 300° | —               | —       | —    | 42      |
|                                  | —    | —               | —       | —    | —       |
|                                  | 350° | —               | 46      | —    | —       |
|                                  | 400° | —               | —       | —    | 47      |
|                                  | 500° | —               | 8       | —    | 23      |
|                                  |      | —               | —       | —    | 23      |

To determine the effective removal of n-heptyl mercaptan or thiophene removal from a naphtha feedstock at liquid phase sulfur removal conditions for manganese oxide and zinc oxide, 50 parts per million (ppm) sulfur as thiophene in naphtha and 50 ppm sulfur as n-heptyl mercaptan and naphtha were passed through a liquid phase sulfur removal zone at various temperatures. The results of such testing is given in FIG. 5.

It is clear that neither manganese oxide nor zinc oxide are particularly effective in removing thiophene from a naphtha feedstock. However, it was surprisingly found that manganese oxide was significantly superior to zinc oxide at removing n-heptyl mercaptan at temperatures in the range of about 400° F. to about 600° F.

The embodiments of this invention in which an exclusive property or privilege is claimed are defined as follows:

1. A reforming process for a hydrocarbon material containing a sulfur component comprising: contacting in a liquid phase sulfur removal zone at liquid phase sulfur removal conditions, said hydrocarbon material with a manganese-containing composition which comprises a manganese component capable of removing at least a portion of said sulfur component at said sulfur removal conditions to produce a reduced sulfur-containing hydrocarbon feedstock, and contacting in a

reforming zone in the presence of hydrogen at hydrocarbon reforming conditions said feedstock with a catalyst comprising a catalytically effective amount of a platinum-group metal component capable of reforming said feedstock at such reforming conditions to produce a reformed product.

2. The process of claim 1 wherein the catalyst also comprises a catalytically effective amount of a halogen component.

3. The process of claim 1 wherein said manganese component comprises an oxide of manganese.

4. The process of claim 3 wherein said oxide of manganese comprises manganous oxide.

5. The process of claim 1 wherein the platinum-group metal component comprises platinum.

6. The process of claim 1 wherein the percent by weight of said manganese component calculated as manganous oxide and based upon the total weight of said manganese-containing composition is in the range of about 35% to about 99% by weight.

7. The process of claim 1 wherein said sulfur removal conditions comprise a temperature below the critical temperature of said hydrocarbon material and a pressure sufficient to maintain the presence of a liquid phase in the sulfur removal zone.

8. The process of claim 7 wherein said sulfur removal conditions comprise a temperature in the range of about 400° to about 600° F. and a pressure from about 100 to about 800 psig wherein said temperature and pressure are selected so as to maintain the presence of a liquid phase.

9. The process of claim 1 wherein said catalyst in the reforming zone also comprises a catalytically effective amount of rhenium.

10. The process of claim 2 wherein the platinum-group metal component, calculated on an elemental basis, is about 0.01% to about 3% by weight of the catalyst and the halide component, calculated on an elemental basis, is about 0.1% to about 5% by weight of the catalyst.

11. The process of claim 1 wherein at least a portion of the manganese-containing composition is in the form of particles each of which have an overall average diameter in the range of about  $\frac{1}{2}$  inch to about 1/32 inch.

20 12. The process of claim 1 wherein the manganese-containing composition comprises at least one component selected to the group consisting of a clay, graphite, alumina, zirconia, chromia, magnesia, curia, boria, silica-alumina, silica-magnesia, chromium-alumina, alumina-boria, alumina-silica-boron phosphate, silica-zirconium, and a combination of alumina and silica.

\* \* \* \* \*

30

35

40

45

50

55

60

65